# EUROPEAN PATENT SPECIFICATION

(11) **EP 1 940 607 B1**
(45) Date of publication and mention of the grant of the patent: **31.12.2008**
(21) Application number: 06803213.5
(22) Date of filing: 11.09.2006
(51) Int. Cl.: B31C 3/00

(54) **SPIRALLY WOUND TUBE WITH VOIDS AND METHOD FOR MANUFACTURING THE SAME**
SPIRALFÖRMIG GEWICKELTE RÖHRE MIT LEERRÄUMEN UND HERSTELLUNGSVERFAHREN DAFÜR
TUBE ENROULE EN SPIRALE COMPORTANT DES CAVITES ET PROCEDE DE FABRICATION

(30) Priority: 13.09.2005 US 225547
(43) Date of publication of application: 09.07.2008
(73) Proprietor: Sonoco Development, Inc., Hartsville, South Carolina 29550 (US)
(72) Inventor: VAN DE CAMP, Johannes, Wilhelmus, Hartsville, SC 29550 (US)
(74) Representative: MacDougall, Alan John Shaw
(86) International application number: PCT/US2006/035049
(87) International publication number: WO 2007/033017

(56) References cited:
- EP-A- 1 459 876
- GB-A- 191 009 498
- US-A1- 2004 144 885

## Description

### FIELD OF INVENTION

The present invention relates generally to paperboard tube structures. More particularly, the invention relates to paperboard tube structures having a construction promoting an enhanced wall thickness and bending stiffness for a given mass of the tube structure.

### BACKGROUND OF THE INVENTION

Within the paperboard tube industry, it is desirable to minimize the amount of ply material used to manufacture a paperboard tube. Paperboard tube structures are often used in consumer good applications such as paper towel rolls or toilet paper rolls, but they are also used in manufacturing applications such as cores for supporting rolled sheet material or in industrial applications such as forms or templates for columnar structures.

Tube structures must possess structural properties commensurate with their intended applications. Paperboard tube designs and manufacturing procedures preferably should minimize the amount of raw materials needed to achieve the required structural properties for the particular tube structure. By reducing the material needed, the expense of producing the paperboard tube structures will likewise decrease.

The bending stiffness and other strength properties of tube structures depend on a number of factors, including the strength of the individual plies of the tube and the wall thickness of the tube. As a general rule, increasing the wall thickness of a tubular structure will result in a stronger tube. An increase in wall thickness can be brought about by using additional plies and/or using thicker plies. In either case, an additional amount of raw material is required, which increases the cost of the paperboard tube. Tube strength can also be increased by using denser, stronger plies, but such stronger plies are relatively more costly.

Therefore, a need exists for a paperboard tube structure requiring a minimal amount of paperboard material while maintaining adequate tube strength. Furthermore, it would be advantageous for such a structure to be the product of a cost effective process.

### BRIEF SUMMARY OF THE INVENTION

The present invention addresses the above needs and achieves other advantages by providing a spirally wound tube having an intermediate zone defining one or more voids and a method of making such a tube. In general, the tube is made by spirally winding a plurality of plies together. More specifically, a plurality of plies form an intermediate zone in the tube having one or more voids, each void having a radial height substantially equal to the radial height of the intermediate zone.

According to one embodiment of the present invention, the tube includes an inner zone, an outer zone, and an intermediate zone. The inner zone is located radially inwardly and includes at least one inner layer. Each inner layer has at least one inner ply. The inner ply or plies are spirally wound to form the inner layer. Similarly, the outer zone is located radially outwardly and includes at least one outer layer. Each outer layer has at least one outer ply. The outer ply or plies are spirally wound to form the outer layer. The intermediate zone is located between the outer zone and inner zone and includes at least one intermediate layer. Each intermediate layer includes more than one intermediate ply. The intermediate plies are spirally wound with gaps between adjacent plies of that intermediate layer. Moreover, the intermediate layers are radially aligned such that the gaps in every intermediate layer are aligned to each other and form voids. Each void has a thickness or radial height substantially equal to the thickness of the intermediate zone.

The width and thickness of the plies may vary. However, according to one preferred embodiment, the thickness of each inner ply, intermediate ply, and outer ply is substantially equal to each other. The width of each intermediate ply is substantially less than the width of each outer ply and inner ply.

In another embodiment of the present invention, the paper tube includes a plurality of paperboard plies spirally wound about an axis and adhered together to form a tube. The wall of the tube comprises an inner zone, an outward zone, and an intermediate zone. The inner zone is located radially inwardly and comprises at least one inner ply. The outer zone is located radially outwardly and comprises at least one outer ply. The intermediate zone is located between the inner zone and the outer zone and comprises a plurality of intermediate paperboard plies. The intermediate paperboard plies are aligned and wound one atop another such that a void exists between adjacent edges of consecutive turns of the intermediate paperboard plies. The thickness or radial height of each void is substantially equal to the thickness of the intermediate zone.

One aspect of the present invention is a method of constructing a paperboard tube with at least one void in its wall. The method includes spirally winding plies about a forming mandrel to form wall zones. In particular, one or more inner plies are spirally wound to form an inner tube wall zone. Two or more intermediate plies are spirally wound and aligned to form an intermediate wall zone with voids between adjacent edges of consecutive turns of the intermediate plies, wherein the radial height of each void is substantially equal to the radial height of the intermediate tube wall zone. Also, one or more outer plies are spirally wound to form an outer tube wall zone. The plies of the inner, intermediate, and outer wall zones are adhered together to form a tube.

According to another embodiment of the present invention, the method includes providing a plurality of plies. The width of each ply is substantially equal. One or more plies are applied to a forming mandrel with nominal gaps between adjacent edges of consecutive turns of each ply to form an inner tube zone. One or more plies are used to form more than one mini-ply. The width of each mini-ply is substantially less than the width of each ply. The mini-plies are applied in a radially aligned fashion to the forming mandrel with gaps between adjacent edges of consecutive turns of the mini-plies to form an intermediate tube zone with voids. The radial height or thickness of each void is substantially equal to the radial height or thickness of the intermediate tube zone. One or more the plies are applied to the forming mandrel with nominal gaps between adjacent edges of consecutive turns of each ply to form an outer tube zone.

In yet another embodiment, the method includes forming more than one intermediate layer. Each layer is formed by spirally winding a plurality of mini-plies. For example, the method includes forming four mini-plies out of one ply and spirally winding the four mini-plies to form one intermediate layer such that a gap exists between adjacent mini-plies. Further, the mini-plies in a given intermediate layer are radially aligned to form voids. Each void has a radial height substantially equal to a radial height of the entire intermediate zone.

Another aspect of the present invention is the forming of the mini-plies out of the one or more of the plies. The forming of the mini-plies may be accomplished using a variety of methods. For example, according to the preferred embodiment, the method further includes a step of perforating one or more of the plies to facilitate the forming of the mini-plies. More specifically, according to this embodiment, the forming of the mini-plies is accomplished by separating one or more of the plies into mini-plies along a perforation line. Alternatively, the forming of the mini-plies may be accomplished by using a water jet cutter or other means known in the art.

### BRIEF DESCRIPTION OF THE SEVERAL VIEWS OF THE DRAWING(S)

Having thus described the invention in general terms, reference will now be made to the accompanying drawings, which are not necessarily drawn to scale, and wherein:
Figure 1 is a perspective view of a tube according to one embodiment of the present invention, with the outer zone of the tube partially broken away to show the intermediate zone;
Figure 2 is a cross-sectional view of the tube shown in Figure 1 taken substantially along line 2-2, with the outer zone of the tube in place;
Figure 3 is a diagrammatic top elevation of an apparatus for forming a tube as shown in Figures 1 and 2, showing mini-plies and plies being wound onto a forming mandrel;
Figure 4 is a cross-sectional view as in Figure 2 of a tube according to an alternative embodiment of the present invention;
Figure 5 is a partial perspective view of an apparatus for forming the tube as shown in Figure 4; and
Figure 6 is an axial cross-sectional view of a portion of the apparatus and plies shown in Figure 5 taken along line 6-6;
Figure 7 is a cross-sectional view as in Figure 2 of a tube according to another alternative embodiment of the present invention; and
Figure 8 is a cross-sectional view as in Figure 2 of a tube according to yet another alternative embodiment of the present invention.

### DETAILED DESCRIPTION OF THE INVENTION

The present invention now will be described more fully hereinafter with reference to the accompanying drawings, in which some but not all embodiments of the invention are shown. Indeed, this invention may be embodied in many different forms and should not be construed as limited to the embodiments set forth herein; rather, these embodiments are provided so that this disclosure will satisfy applicable legal requirements. Like numbers refer to like elements throughout.

Figures 1 and 2 show a spirally wound tube **10** in accordance with one embodiment of the invention. The tube **10** has an inner zone **20,** an intermediate zone **30**, and an outer zone **40.** Each zone **20, 30, 40** comprises one or more layers **120, 130, 140** (each zone in the Figure 1 and 2 having only one layer), and each layer in turn comprises one or more plies or mini-plies. More specifically, the inner zone **20** is located inwardly and radially extends from (and thus defines) the inner diameter of the tube **10** to the intermediate zone **30.** The intermediate zone **30** radially extends from the inner zone **20** to the outer zone **40.** The outer zone **40** is located outwardly and radially extends from the intermediate zone **30** to (and thus defines) the outer diameter of the tube **10.** The layer **130** of the intermediate zone **30** is different than the layers **120, 140** in either the inner or outer zones **20, 40.** The layer **130** of the intermediate zone **30** comprises a plurality of plies that have gaps between consecutive turns of a ply or adjacent plies. In contrast, each of the layers **120, 140** of the inner zone **20** or outer zone **40** comprises only one ply wound with no substantial gaps, as further described below.

As used herein, a "layer" is a region of the tube **10** delimited by an outer radius **rₒ** and an inner radius **rᵢ** that respectively correspond to an outer surface and inner surface of a "ply" of that layer. A "ply" is a unitary sheet of material that, when wound into the tube **10,** constitutes at least a part of a single layer of the tube **10.** Thus, in accordance with the present invention, a layer can comprise more than one ply occupying the region bound by **rₒ** and **rᵢ** as best seen in Figure 2.

According to one embodiment of the present invention and as shown in Figures 1 and 2, the inner zone **20** includes one layer **120** comprising one ply also referred to herein as an inner ply **1020** due to its location within the inner zone **20.** The inner ply **1020** is wound so that nominally it has no substantial gaps between its adjacent edges along the length ofthe tube **10** as generally described in U.S. Patent Number 6,851,643 to Qiu et al. and assigned to the same assignee as the present application, the entire contents of which are hereby incorporated by reference. "Nominally" means that the objective is to wind the inner ply **1020** so that a perfect butt joint exists between the adjacent edges. However, in practice, a perfect butt joint may not always be achieved, and typically small gaps are inadvertently created between the edges of the ply **1020.** In general, such inadvertent gaps will be relatively small compared to the width of the plies.

Similarly, the outer zone **40** includes one layer **140** comprising one ply also referred to herein as an outer ply **1040** due to its location within the outer zone **40.** The outer ply **1040** is wound so that nominally it has no substantial gaps between its adjacent edges along the length of the tube **10.**

It should also be noted, as further described in U.S. Patent Number 6,851,643, it is known from geometrical considerations applicable to spiral winding that to achieve a perfect butt joint, the width of ply, the diameter of the ply, and the spiral wind angle are related. Basically, the width, the angle, or both must increase as the diameter of the ply increases. Therefore, one in the art would appreciate that either the spiral wind angle, the width of the ply, or both may vary between layers to account for the above-mentioned geometrical considerations.

The intermediate zone **30** has one layer **130** comprising more than one mini-ply. For example purposes only and as seen in Figures 2 and 3, the intermediate layer **130** has four mini-plies **1031, 1032, 1033, 1034.** The mini-plies **1031, 1032, 1033, 1034** are wound so a gap **135** is intentionally created between the mini-plies **1031, 1032, 1033, 1034** as best seen in Figure 2. Preferably, for reasons explained further below, the four mini-plies **1031, 1032, 1033, 1034** are formed from a ply **1030** similar to the inner ply **1020** and the outer ply **1040.** Each mini-ply **1031, 1032, 1033, 1034** has a width substantially less than the widths of the inner ply **1020** or the outer ply **1040.** Also each gap **135** between mini-plies **1031, 1032, 1033, 1034** is substantially equal to the width ofthe mini-plies **1031, 1032, 1033, 1034.**

In an alternative embodiment, shown in Figures 4 and 5, the intermediate zone **30** has more than one intermediate layer. Although depicted in the figures as four intermediate layers **130, 230, 330, 430,** the number of layers may vary. Each intermediate layer has more than one mini-ply. Again, for example purposes only, each intermediate layer **130, 230, 330, 430** may have four mini-plies **1030, 1031, 1032, 1033, 2030, 2031, 2032, 2033, 3030, 3031, 3032, 3033, 4030, 4031, 4032, 4033** intentionally wound so a gap **135, 235, 335, 435** is created between adjacent mini-plies in each layer. Also, the mini-plies in each intermediate layer **130, 230, 330, 430** are radially aligned with those of the other intermediate layers as best seen in Figure 4. By radially aligning the mini-plies in the intermediate layers **130**, **230, 330, 430,** the gaps **135, 235, 335, 435** in each layer **130, 230, 330, 430** are aligned, forming voids **35** of larger radial height. More particularly, each void **35** has a radial height or thickness substantially equal to the radial height of the intermediate layers **130, 230, 330, 430** combined (i.e., the height of the intermediate zone **30**). In theory, the radial height of each void **35** should be equal to the combined height of the intermediate layers **130, 230, 330, 430.** However, in practice, the inner layer **120** or the outer layer **140** may sag into a void **35** or a void **35** may be partially filled with an adhesive.

Figure 7 illustrates yet another embodiment of the present invention. According to this embodiment, the inner zone **20** includes three layers **120, 220, 320.** Each inner layer in turn includes one ply **1020, 2020, 3020.** The outer zone **40** includes four layers **140, 240, 340, 440.** Each outer layer in turn includes one ply **1040, 2040, 3040, 4040.** The intermediate zone **30** includes two layers **130, 230.** Each intermediate layer includes four mini-plies **1030, 1031,1032, 1033, 2030, 2031, 2032, 2033.** Between each adjacent mini-ply of an intermediate layer is a gap **135** approximately equal to the width of a mini-ply. Also, as described above, the intermediate layers **130, 230** are radially aligned, forming voids **35.** The wound tube **10** according to this embodiment is referred to in the present specification and appended claims as a "4-spoke core" due to the number of mini-plies per intermediate layer.

Figure 8 illustrates another alternative embodiment of the present invention. According to this embodiment, the inner zone **20** has three layers **120, 220, 320.** The outer zone **40** has four layers **140, 240, 340, 440.** Each layer of the inner zone and outer zone includes one ply **1020, 2020, 3020, 1040, 2040, 3040**, **4040.** The intermediate zone **30** includes two layers **130, 230.** Each intermediate layer includes two mini-plies **1030,1031, 2030, 2031.** A wound tube **10** according to Figure 8 is referred to in the present specification and appended claims as a "2-spoke core" due to the number of mini-plies per intermediate layer.

Wound tubes **10** having either the above-described 2-spoke core or the above-described 4-spoke core were constructed and tested for inner diameter stiffness. One in the art would appreciate that inner diameter stiffness is generally the resistance of the inner diameter to changes to its size due to radial pressure applied to the outer diameter. Inner diameter stiffness is described in more detail in U.S. Patent Number 6,851,643 to Qiu et al. Typically, inner diameter stiffness is measured by psi per 0.001 inches, i.e., how much psi is required on the outer diameter to change the inner diameter by 0.001 inches.

The tested 4-spoke cores were constructed according to Figure 7. In particular, each ply **1020, 2020, 3020, 1040, 2040, 3040, 4040** of the inner and outer layers was approximately 5 inches wide. Each mini-ply **1030,1031,1032, 1033, 2030, 2031, 2032, 2033** of the intermediate layers was approximately 5/8 inches wide. Also, each gap between adjacent mini-plies was approximately 5/8 inches wide. Therefore, the total width of the four mini-plies including the in-between gaps was approximately equal to the width of the plies in the outer and inner layers.

The tested 2-spoke cores were constructed according to Figure 8. Specifically, each ply in the outer and inner layers was approximately 5 inches wide. Each mini-ply of the intermediate layers was approximately 1 ¼ inches wide. Each gap **135** between adjacent mini-plies was approximately 1 ¼ inches wide. Therefore the total width of the two mini-plies including the in-between gaps **135** was approximately equal to the width of the plies in the outer and inner layers.

One in the art would appreciate that the tested 4-spoke cores and 2-spoke cores as generally described-above have substantially the same weight and substantially the same amount of volume of voids. However the test results, shown in the table below, indicated that the 2-spoke cores had a higher inner diameter stiffness.

| **Core type** | **2 spoke** | **4 spoke** | **units** |
|---|---|---|---|
| ID | 3.025 | 3.028 | inch |
| Wall | 0.180 | 0.190 | inch |
| ID stiffness | 50+ | 35 | psi/0.001" |

| | | | |
|---|---|---|---|
| (The test results take into account an 8% moisture content within the tubes.) | | | |

Another embodiment ofthe 2-spoke core was tested against a solid core. In general, a solid core, as referred to within this present specification and appended claims, is a conventional tube constructed without any mini-plies or significant gaps or voids between adjacent plies. However the solid core is constructed generally with the same material as the 2-spoke core and has substantially the same inner diameter and outer diameter. The 2-spoke cores and the solid cores were tested for inner diameter stiffness.

The results of the test are shown in the following table:

| **Core type** | **2 spoke** | **solid** | **units** |
|---|---|---|---|
| ID | 3.078 | 3.073 | inch |
| Wall | 0.331 | 0.336 | inch |
| Weight | 39.31 | 48.71 | grams |
| ID stiffness | 110 | 53 | psi/0.001" |

| | | | |
|---|---|---|---|
| (Again, the test results take into account an 8% moisture content.) | | | |

The results show that the 2-spoke core outperformed the solid core in inner diameter stiffness. Also, as indicated, the 2-spoke core is approximately 20% lower in weight compared to a solid core.

Another aspect of the present invention is a method or process of forming the tube **10.** In general, the tube **10** is formed by spirally winding a plurality of plies about a mandrel **100,** adhering the plies together, and severing portions or sections of the spirally wound plies to form individual tubes **10.** Figure 3 illustrates one method of making the paper tube **10** according to one embodiment of the present invention. Three plies **1020, 1030, 1040** are drawn from respective creels (not shown) and routed along a path to the mandrel **100** by a series of guides. Each ply may have an adhesive applied to it at an adhesive applying station such as a glue pot. For example and as shown, adhesive is applied to the outwardly facing surface of the inner ply **1020** using an adhesive applicator **110** and the inner ply **1020** is spirally wound about the mandrel **100.** A ply **1030** is provided for the intermediate layer **130.** More specifically, the intermediate ply **1030** is routed toward the mandrel **100.** Before the mandrel **100** but preferably after an adhesive applying station, the intermediate ply **1030** is separated into two or more mini-plies at a separation station **115.** For example and as shown, the intermediate ply **1030** is split into four mini-plies **1031, 1032, 1033, 1034.** Each mini-ply **1031, 1032, 1033, 1034** is routed to the mandrel **100** by a series of guides and spacers **107** to ensure proper alignment. The mini-plies **1031, 1032, 1033, 1034** are spirally wound around the mandrel **100** with gaps **135** between adjacent mini-plies **1031, 1032, 1033, 1034.** Next, the outer ply **1040** is spirally wound around the mandrel **100** forming a continuous paper tube **15.** A cut-off station (not shown) may be included to cut the continuous tube **15** into discrete lengths to form individual tubes **10.** A winding belt **101** rotates the continuous tube **15** in a screw fashion such that the tube **15** advances down the mandrel **100.**

As shown in Figures 5 and 6, the method may also include forming more than one intermediate layer **130, 230, 330, 430.** When forming more than one intermediate layer **130, 230, 330, 430,** the mini-plies **1030-1033, 2030-2033, 3030-3033, 4030-4033** of each layer **130, 230, 330, 430** are radially aligned so the gaps **135** of each layer **130, 230, 330, 430** form voids **35.** Each void **35** has a radial height substantially equal to the combined radial height of the intermediate layers **130, 230, 330, 430.** Radially aligning the mini-plies **1030-1033, 2030-2033, 3030-3033,4030-4033** may be accomplished as shown in Figure 5. The mini-plies formed from one ply may form one intermediate layer, and then the next layer of mini-plies formed from another ply may form the next intermediate layer, with the mini-plies from each layer stacked or aligned on each other. Alternatively, the mini-plies formed from one ply may be substantially stacked on top of each other as they are applied to the mandrel **100.** In this alternative embodiment, each intermediate layer may have only one mini-ply.

The forming of mini-plies from one wider ply is one aspect of the present invention. This can be accomplished in several ways, for example with the use of water jet cutting. However, the preferred method is by perforating the plies. More specifically, one or more perforation lines, as best seen in Figures 3 and 5, are made in a ply. The perforating lines facilitate the separating or dividing of the ply into mini-plies. Perforating the ply can occur anywhere in the process, including at the paper mill. However, it is preferred for the separation of the plies into mini-plies to occur near the mandrel **100** and after the adhesive applying station **110.** The wider body of the ply compared to the mini-plies makes it easier to ship, store, and process the perforated ply before it is separated into mini-plies (i.e., the wide perforated ply can be handled as an ordinary non-perforated ply and then can be separated into mini-plies just before winding onto the mandrel).

Many modifications and other embodiments of the invention set forth herein will come to mind to one skilled in the art to which this invention pertains having the benefit of the teachings presented in the foregoing descriptions and the associated drawings. Therefore, it is to be understood that the invention is not to be limited to the specific embodiments disclosed and that modifications and other embodiments are intended to be included within the scope of the appended claims. Although specific terms are employed herein, they are used in a generic and descriptive sense only and not for purposes of limitation.

## Claims

1. A spirally wound tube (10), comprising:
an inner zone (20), an outer zone (40), and an intermediate zone (30),
the inner zone being located radially inwardly and including at least one inner layer (120), each inner layer including at least one inner ply (1020), each inner ply having a width and thickness and being spirally wound;
the outer zone being located radially outwardly and including at least one outer layer (140), each outer layer including at least one outer ply (1040), each outer ply having a width and thickness and being spirally wound; and
the intermediate zone being located between the outer zone and the inner zone and including a plurality of intermediate layers (130), each intermediate layer including at least one interniediate ply (1030), each intermediate ply having a width and thickness and being spirally wound with gaps between adjacent edges of the intermediate ply;
wherein the intermediate plies of the intermediate layers are aligned such that the gaps in every intermediate layer are aligned to each other and form voids, each void having a thickness substantially equal to the thicknesses of the intermediate zone.

2. The tube according to Claim 1, wherein the width of each inner ply is approximately equal to the width of each outer ply and the width of each intermediate ply is substantially less than the width of the inner and outer plies.

3. The tube according to Claim 1, wherein the thickness of each immediate ply, the thickness of each inner ply, and the thickness of each outer ply are substantially equal.

4. The tube according to Claim 1, wherein each intermediate layer comprises four intermediate plies.

5. The tube according to Claim 1, wherein the inner, outer, and intermediate plies comprise paperboard plies.

6. The tube according to Claim 1, wherein each gap in the intermediate zone defines a width and the width of each gap is substantially equal to the width of each intermediate ply.

7. The tube according to Claim 1, where the width of the intermediate plies is substantially one fourth the width of the outer ply or plies.

8. A method of constructing a tube defining at least one void within a cylindrical wall of the tube, the method comprising:
spirally winding from one to a plurality of inner plies about a forming mandrel to form an inner tube wall zone on the mandrel;
spirally winding and aligning a plurality of intermediate plies about the inner tube wall zone on the forming mandrel to form an intermediate tube wall zone with gaps between adjacent edges of consecutive turns of the intermediate plies so as to form voids in the intermediate tube wall zone, wherein the radial height of each void is substantially equal to the radial height of the intermediate tube wall zone;
spirally winding from one to a plurality of outer plies about the intermediate tube wall zone on the forming mandrel to form an outer tube wall zone; and
adhering the contiguous plies together to form a tube.

9. The method according to Claim 8, further comprising:
providing a plurality of plies, each ply defining a first width, wherein the first width of every ply is approximately equal;
spirally winding one or more of the plies about the forming mandrel with substantially zero gaps between adjacent edges of consecutive turns of each ply to form the inner tube wall zone;
forming a plurality of mini-plies out of one or more of the plies, each mini-ply having a second width less than the first width; and
spirally winding the plurality of mini-plies in a radially layered and aligned fashion about the forming mandrel with gaps between adjacent edges of consecutive turns of the mini-plies to form the intermediate tube wall zone.

10. The method according to Claim 9, further including the step of perforating one or more of the plies to facilitate the forming of the mini-plies, wherein the forming of the mini-plies includes separating one or more of the plies along a perforation in the plies.

11. The method according to Claim 9, wherein the forming of the mini-plies further includes using water jet cutting to separate one or more of the plies into min-plies.

12. The method according to Claim 9, wherein four mini-plies are made from one ply and are spirally wound to shape one intermediate layer.

13. The method according to Claim 12, wherein the mini-plies in each intermediate layer are spirally wound such that each gap between adjacent mini-plies is approximately equal to a width of a mini-ply.

14. The method according to Claim 9, comprising the steps of:
drawing a continuous ply from a supply and advancing the ply along a path toward the forming mandrel; and
dividing the ply into a plurality of partial-width plies at a dividing station located along the path so as to form the mini-plies.

15. The method according to Claim 14, further comprising the step of advancing the mini-plies from the dividing station to the forming mandrel and spirally winding the mini-plies about the forming mandrel, such that the drawing, dividing, and spirally winding steps comprise a continuous process.

## Patentansprüche

1. Spiralgewickeltes Rohr bzw. spiralförmig gewundene Röhre (10) das bzw. die aufweist:
eine innere Zone (20), eine äußere Zone (40), und eine mittlere bzw. dazwischen liegende Zone (30),
die innere Zone ist radial nach innen angeordnet und schließt zumindest eine innere Schicht (120) ein, wobei jede innere Schicht zumindest eine innere Lage (1020) einschließt, wobei jede innere Lage eine Breite und Dicke aufweist und spiralgewickelt bzw. spiralförmig gewunden ist;
die äußere Zone ist radial nach außen angeordnet und schließt zumindest eine äußere Schicht (140) ein, wobei jede äußere Schicht zumindest eine äußere Lage (1040) einschließt, wobei jede äußere Lage eine Breite und Dicke aufweist und spiralgewickelt bzw. spiralförmig gewunden ist; und
die mittlere bzw. dazwischen liegende Zone ist zwischen der äußere Zone und der inneren Zone angeordnet und schließt eine Vielzahl von mittleren Schichten bzw. dazwischen liegenden Schichte (130) ein, wobei jede mittlere bzw. dazwischen liegende Schicht zumindest eine mittlere bzw. dazwischen liegende Lage (1030) einschließt, wobei jede mittlere bzw. dazwischen liegende Lage eine Breite und Dicke aufweist und spiralgewickelt bzw. spiralförmig gewunden ist, und zwar mit Lücken zwischen angrenzenden Flanken bzw. Kanten der mittleren bzw. dazwischen liegenden Lage;
wobei die mittleren bzw. dazwischen liegenden Lagen der mittleren bzw. dazwischen liegenden Schichten derart ausgerichtet sind, dass die Lücken in jeder mittleren bzw. dazwischen liegenden Schicht zueinander ausgerichtet sind und Auslassungen bzw. Lücken oder Hohlräume ausbilden, wobei jede Auslassung bzw. Lücke oder jeder Hohlraum eine Dicke aufweist, die im Wesentlichen gleich zu der Dicke der mittleren bzw. dawischen liegenden Zone ist.

2. Rohr bzw. Röhre nach Anspruch 1, wobei die Breite von jeder inneren Lage ungefähr gleich zu der Breite von jeder äußeren Lage ist und die Breite von jeder mittleren bzw. dazwischen liegenden Lage im Wesentlichen weniger bzw. kleiner als die Breite der inneren und äußeren Lagen ist.

3. Rohr bzw. Röhre nach Anspruch 1, wobei die Dicke von jeder mittleren bzw. dazwischen liegenden Lage, die Dicke von jeder inneren Lage und die Dicke von jeder äußeren Lage im Wesentlichen gleich sind.

4. Rohr bzw. Röhre nach Anspruch 1, wobei jede mittlere bzw. dazwischen liegende Schicht weiter vier mittlere bzw. dazwischen liegende Lagen aufweist.

5. Rohr bzw. Röhre nach Anspruch 1, wobei die innere, äußere und mittlere bzw. dazwischen liegende Lagen Lagen aus Pappe bzw. Kartonlagen aufweisen.

6. Rohr bzw. Röhre nach Anspruch 1, wobei jede Lücke in bzw. bei der mittleren bzw. dazwischen liegenden Zone eine Breite definiert und die Breite von jeder Lücke im Wesentlichen gleich zu der Breite von jeder mittleren bzw. dazwischen liegenden Lage ist.

7. Rohr bzw. Röhre nach Anspruch 1, wobei die Breite der mittleren bzw. dazwischen liegenden Lagen im Wesentlichen ein viertel der Breite der äußeren Lage oder Lagen ist.

8. Verfahren zum Konstruieren eines Rohres bzw. einer Röhre, das bzw. die zumindest eine Auslassung bzw. eine Lücke oder einen Hohlraum innerhalb einer zylindrischen Wand des Rohres bzw. der Röhre definiert, wobei das Verfahren aufweist:
um einen Ausbildungsdorn bzw. eine Ausbildungsspindel werden spiralförmig von einer zu einer Vielzahl von inneren Lagen gewickelt, um eine innere Rohrwandzone bzw. Röhrenwandzone auf dem Dom bzw. der Spindel auszubilden;
um die inneren Rohrwandzone bzw. Röhrenwandzone auf dem Ausbildungsdorn bzw. der Ausbildungsspindel werden spiralförmig gewickelt und ausgerichtet eine Vielzahl von mittleren bzw. dazwischen liegenden Lagen, um eine mittlere bzw. dazwischen liegende Rohrwandzone bzw. Röhrenwandzone mit Lücken zwischen angrenzenden Flanken bzw. Kanten von aufeinander folgenden Umdrehungen bzw. Umläufen oder Drehungen der mittleren bzw. dazwischen liegenden Lagen auszubilden, um so Auslassungen bzw. Lücken oder Hohlräume in bzw. bei der mittleren bzw. dazwischen liegenden Rohrwandzone bzw. Röhrenwandzone auszubilden, wobei die radiale Höhe von jeder Auslassung bzw. Lücke oder jedem Hohlraum im Wesentlichen gleich zu der radialen Höhe der mittleren bzw. dazwischen liegenden Rohrwandzone bzw. Röhrenwandzone ist;
um die mittlere bzw. dazwischen liegende Rohrwandzone bzw. Röhrenwandzone auf dem Ausbildungsdorn bzw. der Ausbildungsspindel werden spiralgewickelt bzw. spiralförmig gewickelt von einer zu einer Vielzahl von äußeren Lagen, um eine äußere Rohrwandzone bzw. Röhrenwandzone auszubilden; und
die kontinuierlichen Lagen werden zusammen angeheftet bzw. geklebt oder verbunden, um ein Rohr bzw. eine Röhre auszubilden.

9. Verfahren nach Anspruch 8, weiter aufweisend:
eine Vielzahl von Lagen wird bereitgestellt, wobei jede Lage eine erste Breite definiert, wobei die erste Breite von jeder Lage ungefähr gleich ist;
eine oder mehrere der Lagen werden spiralgewickelt bzw. spiralförmig gewickelt, und zwar um den Ausbildungsdorn bzw. die Ausbildungsspindel, und zwar mit im Wesentlichen null Lücken zwischen angrenzenden Flanken bzw. Kanten von aufeinander folgenden Umdrehungen bzw. Umläufen oder Drehungen von jeder Lage, um die innere Rohrwandzone bzw. Röhrenwandzone auszubilden;
eine Vielzahl von Mini-Lagen von der einen oder der mehreren Lagen werden ausgebildet, wobei jede Mini-Lage eine zweite Breite aufweist, die kleiner als die erste Breite ist; und
die Vielzahl von Mini-Lagen werden in einer radial geschichteten und ausgerichteten Weise um den Ausbildungsdorn bzw. die Ausbildungsspindel mit Lücken zwischen angrenzenden Kanten bzw. Flanken der aufeinander folgenden Umdrehungen bzw. Umläufe Drehungen der Mini-Lagen spiralgewickelt bzw. spiralförmig gewickelt, um die mittleren bzw. dazwischen liegende Rohrwandzone bzw. Röhrenwandzone auszubilden.

10. Verfahren nach Anspruch 9, weiter einschließend den Schritt des Perforierens eine oder mehrere der Lagen, um das Ausbilden der Mini-Lagen zu erleichtern, wobei das Ausbilden der Mini-Lagen das Separieren bzw. Trennen einer oder mehrere der Lagen entlang der Perforation in bzw. bei den Lagen einschließt.

11. Verfahren nach Anspruch 9, wobei das Ausbilden der Mini-Lagen weiter die Verwendung des Wasserstrahlschneidens einschließt, um eine oder mehrere der Lagen in Mini-Lagen zu separieren bzw. zu trennen.

12. Verfahren nach Anspruch 9, wobei vier Mini-Lagen aus einer Lage gemacht werden und spiralgewickelt bzw. spiralförmig gewickelt werden, um eine mittlere bzw. dazwischen liegende Schicht zu formen bzw. zu gestalten.

13. Verfahren nach Anspruch 12, wobei die Mini-Lagen in jeder mittleren bzw. dazwischen liegenden Lage spiral gewickelt bzw. spiralförmig gewickelt werden, und zwar derart, dass jede Lücke zwischen angrenzenden Mini-Lagen ungefähr gleich zu einer Breite einer Mini-Lage ist.

14. Verfahren nach Anspruch 9, aufweisend die Schritte:
ein kontinuierliche Lage wird von einer Zuführung gezogen und die Lage wird weiter entlang eines Pfades zu dem Ausbildungsdorn bzw. der Ausbildungsspindel fortgeführt bzw. gebracht; und
die Lage wird in eine Vielzahl von teil-breiten Lagen geteilt, und zwar bei einer Teilstation bzw. Teilungsstation, die entlang des Pfades angeordnet ist, um so die Mini-Lagen auszubilden.

15. Verfahren nach Anspruch 14, weiter aufweisend den Schritt des Vorwärtsbringens bzw. Weiterführens der Mini-Lage von der Teilstation bzw. Teilungsstation zu dem Ausbildungsdorn bzw. der Ausbildungsspindel und dem Spiralwickeln bzw. spiralförmigen Wickeln der Mini-Lagen um den Ausbildungsdorn bzw. die Ausbildungsspindel, und zwar derart, dass die Schritte des Ziehens, Teilens und spiralförmig Wickelns einen kontinuierlichen Prozess aufweisen.

## Revendications

1. Tube enroulé en spirale (10) comprenant :
une zone intérieure (20), une zone extérieure (40) et une zone intermédiaire (30) ;
la zone intérieure étant située radialement vers l'intérieur et comprenant au moins une couche intérieure (120), chaque couche intérieure comprenant au moins une strate intérieure (1020), chaque strate intérieure ayant une largeur et une épaisseur et étant enroulée en spirale ;
la zone extérieure étant située radialement vers l'extérieur et comprenant au moins une couche extérieure (140), chaque couche extérieure comprenant au moins une strate extérieure (1040), chaque strate extérieure ayant une largeur et une épaisseur et
étant enroulée en spirale ; et
la zone intermédiaire étant située entre la zone extérieure et la zone intérieure et
comprenant une pluralité de couches intermédiaires (130), chaque couche intermédiaire comprenant au moins une strate intermédiaire (1030), chaque strate intermédiaire ayant une largeur et une épaisseur et étant enroulée en spirale avec des espaces entre les bords adjacents de la strate intermédiaire ;
dans lequel les strates intermédiaires des couches intermédiaires sont alignées de telle sorte que les espaces dans chaque couche intermédiaire soient alignés les uns avec les autres et forment des vides, chaque vide ayant une épaisseur sensiblement égale aux épaisseurs de la zone intermédiaire.

2. Tube selon la revendication 1, dans lequel la largeur de chaque strate intérieure est approximativement égale à la largeur de chaque strate extérieure et la largeur de chaque strate intermédiaire est sensiblement inférieure à la largeur des strates intérieure et extérieure.

3. Tube selon la revendication 1, dans lequel l'épaisseur de chaque strate intermédiaire, l'épaisseur de chaque strate intérieure et l'épaisseur de chaque strate extérieure sont sensiblement égales.

4. Tube selon la revendication 1, dans lequel chaque couche intermédiaire comprend quatre strates intermédiaires.

5. Tube selon la revendication 1, dans lequel les strates intérieure, extérieure et intermédiaire comprennent des strates de carton.

6. Tube selon la revendication 1, dans lequel chaque espace dans la zone intermédiaire définit une largeur et la largeur de chaque espace est sensiblement égale à la largeur de chaque strate intermédiaire.

7. Tube selon la revendication 1, dans lequel la largeur des strates intermédiaires est sensiblement d'un quart de la largeur de la strate ou des strates extérieure(s).

8. Procédé de construction d'un tube définissant au moins un vide dans une paroi cylindrique du tube, le procédé comprenant :
l'enroulement en spirale d'une à plusieurs strates intérieures autour d'un mandrin de formage pour former une zone de paroi de tube intérieure sur le mandrin ;
l'enroulement en spirale et l'alignement d'une pluralité de strates intermédiaires autour de la zone de paroi de tube intérieure sur le mandrin de formage pour former une zone de paroi de tube intermédiaire avec des espaces entre les bords adjacents de tours consécutifs des strates intermédiaires de façon à former des vides dans la zone de paroi de tube intermédiaire, dans lequel la hauteur radiale de chaque vide est sensiblement égale à la hauteur radiale de la zone de paroi de tube intermédiaire ;
l'enroulement en spirale d'une à plusieurs strates extérieures autour de la zone de paroi de tube intermédiaire sur le mandrin de formage pour former une zone de paroi de tube extérieure ; et
l'adhérence des strates contiguës ensemble pour former un tube.

9. Procédé selon la revendication 8, comprenant en outre :
la fourniture d'une pluralité de strates, chaque strate définissant une première largeur,
dans lequel la première largeur de chaque strate est approximativement égale ;
l'enroulement en spirale d'une ou de plusieurs des strates autour du mandrin de formage avec sensiblement aucun espace entre les bords adjacents de tours consécutifs de chaque strate pour former la zone de paroi de tube intérieure ;
la formation d'une pluralité de mini-strates à partir d'une ou de plusieurs des strates, chaque mini-strate ayant une seconde largeur inférieure à la première largeur ; et
l'enroulement en spirale de la pluralité de mini-strates de façon empilée radialement et alignée autour du mandrin de formage avec des espaces entre les bords adjacents de tours consécutifs des mini-strates pour former la zone de paroi de tube intermédiaire.

10. Procédé selon la revendication 9, comprenant en outre l'étape consistant à perforer une ou plusieurs des strates pour faciliter la formation de mini-strates, dans lequel la formation des mini-strates comprend la séparation d'une ou de plusieurs des strates le long d'une perforation dans les strates.

11. Procédé selon la revendication 9, dans lequel la formation des mini-strates comprend en outre l'utilisation d'une découpe à jet d'eau pour séparer une ou plusieurs des strates en mini-strates.

12. Procédé selon la revendication 9, dans lequel quatre mini-strates sont réalisées à partir d'une strate et sont enroulées en spirale pour former une couche intermédiaire.

13. Procédé selon la revendication 12, dans lequel les mini-strates dans chaque couche intermédiaire sont enroulées en spirale de telle sorte que chaque espace entre les mini-strates adjacentes soit approximativement égal à une largeur d'une mini-strate.

14. Procédé selon la revendication 9, comprenant les étapes consistant à :
tirer une strate continue à partir d'une alimentation et faire avancer la strate le long d'un trajet vers le mandrin de formage ; et
diviser la strate en une pluralité de strates de largeur partielle dans une station de séparation située le long du trajet de façon à former les mini-strates.

15. Procédé selon la revendication 14, comprenant en outre l'étape d'avancement des mini-strates depuis la station de division jusqu'au mandrin de formage et d'enroulement en spirale des mini-strates autour du mandrin de formage, de telle sorte que les étapes de traction, de division et d'enroulement en spirale comprennent un processus continu.
